# EUROPEAN PATENT SPECIFICATION

(11) **EP 3 578 693 B1**
(45) Date of publication and mention of the grant of the patent: **15.04.2020**
(21) Application number: 18176788.0
(22) Date of filing: 08.06.2018
(51) Int. Cl.: C25D 3/60, C25D 7/00

(54) **AQUEOUS COMPOSITION FOR DEPOSITING A TIN SILVER ALLOY AND METHOD FOR ELECTROLYTICALLY DEPOSITING SUCH AN ALLOY**
WÄSSRIGE ZUSAMMENSETZUNG ZUR ABSCHEIDUNG EINER ZINN-SILBER-LEGIERUNG UND VERFAHREN ZUR ELEKTROLYTISCHEN ABSCHEIDUNG SOLCH EINER LEGIERUNG
COMPOSITION AQUEUSE POUR LE DÉPÔT D'UN ALLIAGE D'ARGENT ET D'ÉTAIN ET PROCÉDÉ DE DÉPÔT ÉLECTROLYTIQUE D'UN TEL ALLIAGE

(43) Date of publication of application: 11.12.2019
(73) Proprietor: Atotech Deutschland GmbH, 10553 Berlin (DE)
(72) Inventor: Jha, Himendra, 10553 Berlin (DE); Schmidt, Ralf, 10553 Berlin (DE); Schwarz, Christian, 10553 Berlin (DE); Kocer, Recep, 10553 Berlin (DE); Vazhenin, Grigory, 10553 Berlin (DE)

(56) References cited:
- EP-A1- 1 553 211
- EP-A1- 2 221 396
- US-B1- 6 607 653

## Description

### Field of the Invention

The present invention relates to an aqueous composition for depositing a tin silver alloy, a method for electrolytically depositing such an alloy onto a substrate, and the use of said composition for electrolytically depositing tin silver alloy solder bumps or tin silver alloy solder caps onto pillars.

### Background of the Invention

In modern packaging technologies a clear trend toward decreasing sizes is observed to address increased performance and improved functionality for electronic devices. Solder caps on copper pillars have turned out to be an interesting and promising alternative to conventional solder ball applications, in particular for Flip-Chip applications in microelectronic devices.

Solder caps on copper pillars typically consist of two elements: (i) a structural element made of copper forming the pillar, e.g. a cylinder and (ii) a solder cap on top of said pillar. A large number of such capped copper pillars are typically arranged on a die, which is part of a wafer. Compared to conventional solder ball applications, solder caps on copper pillars provide an improved thermal and electrical behaviour due to the comparatively large volume of copper in the capped pillar, which provides an excellent electrical connection and increased conductivity. The solder cap provides an electrical as well as mechanical connection between the respective pillar and a corresponding feature, for example a pillar of another die.

An additional advantage of solder caps on copper pillars is the slim shape of the pillars compared to ball-like conventional solder ball applications. This allows a reduced distance (also called pitch) between two neighbouring pillars, which is a key element for higher packaging.

The solder cap typically includes tin and in many cases is a tin silver alloy; typically being free of lead. Such an alloy usually provides an excellent solderability and is a suitable alternative to previously used lead-containing solder caps and solder balls, respectively.

Depositing such tin silver alloys is known in the art. For example, JP 2006-265573 A discloses a tin silver alloy plating bath without cyanide, which improves solderability and appearance of an electrodeposition film obtained from the tin silver bath.

EP 0 854 206 B1 relates to an acidic tin silver alloy plating bath, which is substantially free of cyanide, and a method for electroplating tin silver alloy onto a substrate.

US 2014/0251818 A1 refers to a cyanide-free tin alloy plating solution having outstanding serial stability as well as a method of plating tin alloy onto an electroconductive object using the tin alloy plating solution. The tin alloy plating solution contains tin ions and one or more additional metal ions of silver, copper, bismuth, indium, palladium, lead, zinc, or nickel, and peptides with cysteine residues.

WO 03/046260 A2 relates to an electrolysis bath for electrodepositing silver-tin alloys that, in addition to water serving as a solvent with a pH value of less than 1.5, contains a water-soluble silver compound, a water-soluble tin compound and an organic complexing agent. In order to obtain a stable electrolysis bath that enables the homogenous deposition of a compact tin silver alloy with any type of composition, an aliphatic complexing agent having a sulfide group and an amino group is used as a complexing agent, whereby said functional groups are bound to different carbon atoms.

EP 1 553 211 B1 relates to a tin-silver-copper plating solution comprising 30-90 wt% of water, a sulfonic acid, tin ions, copper ions and silver ions, wherein the concentration of the silver ions is 0.01 to 0.1 mol/L, the concentration of the tin ions is 0.21 to 2 mol/L, the concentration of the copper ions is 0.002 to 0.02 mol/L and the mole ratio of the silver-ions to the copper ions is in the range of 4.5 to 5.58.

US 6,607,653 B1 relates to a tin-copper alloy plating bath, tin-copper-bismuth alloy plating bath or tin-copper-silver alloy plating bath containing a soluble metal compound and a specific sulfur-containing compound.

EP 2 221 396 A1 relates to a composition comprising one or more sources of tin ions, one or more sources of alloying metal ions, the metal ions are selected from the group consisting of silver ions, copper ions and bismuth ions, one or more flavone compounds, and one or more compounds having a formula: HOR(R")SR'SR(R")OH wherein R, R' and R" are the same or different and are alkylene radicals having 1 to 20 carbon atoms.

Despite known approaches, depositing a tin silver alloy, typically carried out by means of electrolytic deposition, requires highly sophisticated and accurate deposition methods to obtain solder caps with a high measure of uniformity. Only then the appearance of dendrites on the pillar can be effectively reduced or even completely avoided. Such dendrites are irregular, non-uniform solder caps with the potential to even bridge two adjacent pillars. In such a case the entire die carrying a high number of pillars with solder caps might become useless and needs to be thrown away. Suitable methods and compositions, respectively, to obtain copper pillars with basically dendrite-free solder caps are still missing and highly demanded to decrease the number of defective goods.

### Objective of the present Invention

It is an objective of the present invention to provide an aqueous composition for depositing a tin silver alloy, which overcomes the above mentioned problems. It is in particular an objective to obtain a tin silver alloy with high uniformity such that for example very uniform solder caps on pillars are obtained and dendrites (as defined above) are basically avoided; in particular at comparatively high current densities in the range from 20 A/dm² to 30 A/dm². It is furthermore an objective that said tin silver alloy can also be utilized to form solder bumps having above mentioned advantages.

It is an additional objective of the present invention to provide also a respective method for electrolytically depositing such a tin silver alloy, in particular for electrolytically depositing tin silver alloy solder bumps and tin silver alloy solder caps on pillars such that the occurrence of dendrites is suppressed for both solder caps and solder bumps.

### Summary of the Invention

These objectives are solved by an aqueous composition for depositing a tin silver alloy, the composition comprising
(a) tin ions,
(b) silver ions,
(c) at least one first compound independently selected from the group consisting of unsubstituted bis(aminophenyl)disulfides, substituted bis(aminophenyl)disulfides, unsubstituted dipyridyldisulfides, and substituted dipyridyldisulfides, and
(d) at least one second compound of formula (II) wherein independently
   X denotes a C1 to C10 alkyl moiety comprising one or more than one sulfhydryl group,
   R¹ denotes hydrogen, methyl, ethyl, linear C3 to C5 alkyl, branched C3 to C5 alkyl, unsubstituted phenyl, substituted phenyl, unsubstituted benzyl, or substituted benzyl, and
   R² denotes methyl, ethyl, linear C3 to C5 alkyl, branched C3 to C5 alkyl, unsubstituted phenyl, substituted phenyl, unsubstituted benzyl, or substituted benzyl.

Furthermore, the additional objective is solved by a method for electrolytically depositing a tin silver alloy onto a substrate, the method comprising the steps
(A) providing the substrate,
(B) providing an aqueous composition according to the present invention, preferably as described throughout the text as being preferred,
(C) contacting said substrate with said aqueous composition and supplying an electrical current such that said tin silver alloy is electrolytically deposited onto the substrate.

In addition, the objectives are solved by the use of an aqueous composition according to the present invention, preferably as described as being preferred throughout the present text, for electrolytically depositing tin silver alloy solder bumps or tin silver alloy solder caps onto metal pillars, preferably for electrolytically depositing tin silver alloy solder caps onto copper pillars.

### Brief description of the figure

Figure 1 is a top view of a section of a die comprising a plurality of copper pillars with tin silver solder caps (shown as black dots), obtained according to the present invention. For further details see the examples below in the text. The silicon-based wafer coupon comprising the die is shown in light gray.
Figure 2 is a top view of a section of a die comprising a plurality of copper pillars with tin silver solder caps (shown as black dots), obtained according to prior art (JP 2006-265573 A, see examples below). Again, the silicon-based wafer coupon comprising the die is shown in light gray. In the upper right corner, a dendrite formed on top of a cylindrical copper pillar is emphasized by the letter "A".
Figure 3 is a diagram showing the complexing properties of various compounds for silver ions. On the x-axis the concentration in g/L of the respective compound is given, wherein on the y-axis the overpotential in dependence on the compound's concentration is given. In the figure, letters have the following meaning: A: 2,2'-dithiodianiline, B: 2-(dimethylamino)ethanethiol, C: L-cysteine, D: glutathione, and E: cysteamine.

### Detailed Description of the Invention

Own experiments show that the aqueous composition, the method, and the use as defined above, result in excellent uniform tin silver solder caps. These caps can be excellently utilized for metal pillars, in particular copper pillars (see examples below in the text). Furthermore, the formation of dendrites is impressively decreased or even entirely prevented.

In the context of the present invention, the term "at least one" denotes (and is exchangeable with) "one, two, three or more than three".

The term "independently" denotes for example that in the at least one second compound of formula (II) X, R¹, and R² in a first compound of formula (II) are selected independently from X, R¹, and R² in a second and further compound of formula (II) in the aqueous composition of the present invention. Furthermore, for example the at least one first compound is independently selected from a number of compound groups. This means that, if for example two first compounds are selected, each compound can be selected from a different compound group, for example one compound is a substituted bis(aminophenyl)disulfide, the other is a substituted dipyridyldisulfide. In other words, the selection of the first compound of said two first compounds is independent from the selection of the second first compound of said two first compounds.

The composition of the present invention is an aqueous composition, which means that water is the primary component. Thus, more than 50 wt-% of the aqueous composition is water, based on the total weight of the aqueous composition, preferably at least 60 wt-%, even more preferably at least 70 wt-%, most preferably 80 wt-% or more. It is preferred that the aqueous composition is substantially free of organic solvents; more preferably does not contain organic solvents at all. Furthermore, the aqueous composition is preferably an aqueous solution, i.e. is homogeneous and thus preferably does not contain any particles.

In the context of the present invention, the term "at least" in combination with a particular value denotes (and is exchangeable with) this value or more than this value. For example, "at least 70 wt-%" denotes (and is exchangeable with) "70 wt-% or more than 70 wt-%".

In the context of the present invention, the term "substantially free" of a subject-matter (e.g. a compound, a material, etc.) independently denotes that said subject-matter is not present at all or is present only in (to) a very little and undisturbing amount (extent) without affecting the intended purpose of the invention. For example, such a subject-matter might be added or utilized unintentionally, e.g. as unavoidable impurity. "Substantially free" preferably denotes 0 (zero) ppm to 50 ppm, based on the total weight of the aqueous composition of the present invention, if defined for said aqueous composition, or based on the total weight of the tin silver alloy, if defined for said alloy; preferably 0 ppm to 25 ppm, more preferably 0 ppm to 10 ppm, even more preferably 0 ppm to 5 ppm, most preferably 0 ppm to 1 ppm. Zero ppm denotes that a respective subject-matter is not at all comprised.

Preferred is an aqueous composition of the present invention, wherein the composition is acidic, preferably the composition has a pH in the range from -2 to +4, more preferably in the range from -1 to +2, most preferably in the range from -0.5 to +1.2. Generally, acidic compositions, in particular having a pH range as defined above, are typically free of cyanide, which is desired for environmental reasons. Thus, also the composition of the present invention is preferably free of cyanide. Furthermore, above mentioned pH ranges lead to an improved quality of the deposited tin silver alloy compared to a composition with a pH significantly higher than 4 or even being alkaline. Furthermore, the stability is increased if the pH is in the above defined pH ranges. In particular undesired plate out is observed if the pH is significantly higher than 4 or even alkaline. In order to prevent plate out in compositions having a pH significantly higher than 4 or even alkaline, typically very strong complexing agents are utilized such as environmentally hazardous cyanides. However, this can be successfully avoided in the composition and method of the present invention. As a result, waste water treatment is simplified and environmental issues are prevented. In the context of the present invention, pH is referenced to a temperature of 20°C.

The aqueous composition of the present invention is for depositing a tin silver alloy, preferably a tin silver alloy being substantially free of sulfur.

The aqueous composition of the present invention comprises (a) tin ions and (b) silver ions in order to deposit the tin silver alloy. In the aqueous composition the tin ions are preferably tin (II) ions and the silver ions preferably silver (I) ions.

Preferred is an aqueous composition of the present invention, wherein in the aqueous composition the tin ions are present in a total concentration in the range from 20 g/L to 200 g/L, based on the total volume of the aqueous composition, preferably in the range from 25 g/L to 150 g/L, more preferably in the range from 30 g/L to 120 g/L, even more preferably in the range from 35 g/L to 100 g/L, most preferably in the range from 40 g/L to 90 g/L. A concentration significantly below 20 g/L often results in an undesired low deposition rate. If the concentration significantly exceeds 200 g/L problems with solubility are frequently observed. An optimal compromise of deposition rate and solubility is obtained in above defined preferred concentration ranges. Best results have been obtained with a concentration in the range from 35 g/L to 100 g/L and from 40 g/L to 90 g/L, respectively.

The tin ions are from a tin ion source. The tin ion source of said tin ions is preferably at least one tin salt, more preferably at least one inorganic tin salt and/or at least one organic tin salt. Preferred inorganic tin salts are selected from the group consisting of tin oxide, tin sulfate, and tin sulfide. Preferred organic tin salts are selected from the group consisting of tin acetate, tin citrate, tin oxalate, and tin alkyl sulfonates. More preferred is an aqueous composition of the present invention, wherein the tin ions are from at least one organic tin salt, preferably from at least one tin alkyl sulfonate. In the aqueous composition of the present invention most preferred is tin methane sulfonate. Preferably in each tin ion source tin is present as tin (II).

Preferred is an aqueous composition of the present invention, wherein in the aqueous composition the silver ions are present in a total concentration in the range from 0.1 g/L to 10 g/L, based on the total volume of the aqueous composition, preferably in the range from 0.2 g/L to 8 g/L, more preferably in the range from 0.3 g/L to 6 g/L, even more preferably in the range from 0.4 g/L to 4 g/L, most preferably in the range from 0.5 g/L to 2 g/L. A concentration significantly below 0.1 g/L often results in an insufficient amount of silver in the tin silver alloy leading to undesired mechanical and electrical properties in respective solder caps and solder bumps. If the concentration significantly exceeds 10 g/L the composition is not sufficiently stable and plate out is sometimes observed. In Addition, too much silver is usually incorporated into the tin silver alloy, significantly increasing the melting point of a respective solder cap, which is undesired in subsequent reflow processes. Optimal melting points are obtained in the above defined preferred concentration ranges, most preferably in the ranges from 0.4 g/L to 4 g/L and 0.5 g/L to 2 g/L, respectively.

The silver ions are from a silver ion source. The silver ion source of said silver ions is preferably at least one silver salt, more preferably at least one inorganic silver salt and/or at least one organic silver salt. Preferred inorganic silver salts are selected from the group consisting of silver oxide, silver sulfate, and silver nitrate. Preferred organic silver salts are selected from the group consisting of silver acetate, silver citrate, silver oxalate, and silver alkyl sulfonates. More preferred is an aqueous composition of the present invention, wherein the silver ions are from at least one organic silver salt, preferably from at least one silver alkyl sulfonate. In the aqueous composition of the present invention most preferred is silver methane sulfonate. Preferably in each silver ion source silver is present as silver (I).

Most preferred, the silver ion source as well as the tin ion source comprise alkylsulfonates, more preferably are alkylsulfonates. This is in particular preferred if the pH in the aqueous composition of the present invention is (re)adjusted by means of alkylsulfonic acids. In this case only one type of organic acid anion is present in the composition of the present invention.

Preferred is an aqueous composition of the present invention, wherein the molar ratio of the tin ions to the silver ions is in the range from 200:1 to 5:1, preferably in the range from 150:1 to 10:1, more preferably in the range from 125:1 to 12:1, most preferably in the range from 100:1 to 15:1. If the molar ratio is significantly exceeding 200:1 usually silver is insufficiently incorporated into the tin silver alloy. If the molar ratio is significantly below 5:1 in some cases the tin silver alloy comprises too much silver. However, if the molar ratio is as defined above, in particular in the range from 125:1 to 12:1 and from 100:1 to 15:1, respectively, an excellent uniform tin silver alloy is obtained and dendrites are very much suppressed in solder caped pillars.

Very preferred is a composition of the present invention, wherein the composition is substantially free of, preferably does not comprise, halide ions, most preferably chloride ions. First, silver chloride is very insoluble in an aqueous environment. Second, it has been observed in some cases that in particular chloride ions, although present in low amounts and not necessarily leading to immediate precipitation of insoluble chlorides, result in deposition defects in the tin silver alloy. Thus, it is preferred to not utilize tin ion sources and silver ion sources comprising halide anions, most preferably chloride ions.

In some cases an aqueous composition of the present invention is preferred, wherein the composition additionally comprises copper (II) ions, preferably in a total concentration from 0.06 g/L to 5 g/L, based on the total volume of the aqueous composition, more preferably in a total concentration from 0.3 g/L to 4 g/L, even more preferably in a total concentration from 0.8 g/L to 3 g/L. Such a composition is for basically depositing a tin silver copper alloy.

In some of these cases an aqueous composition of the present invention is preferred, wherein the composition comprises copper (II) ions in a total concentration from 0.06 g/L to 0.6 g/L, based on the total volume of the aqueous composition, preferably from 0.2 g/L to 0.5 g/L, more preferably from 0.3 g/L to 0.4 g/L. In such cases copper is incorporated into the tin silver alloy only to a very limited extent.

In alternative cases an aqueous composition of the present invention is preferred, wherein the composition comprises copper (II) ions in a total concentration from 0.7 g/L to 5 g/L, based on the total volume of the aqueous composition, preferably from 1 g/L to 4.2 g/L, more preferably from 1.3 g/L to 3.6 g/L, even more preferably from 2.1 g/L to 3.1 g/L. In such cases copper is incorporated into the tin silver alloy to a more significant extent.

However, in most cases it is in particular desired to not include copper ions in the aqueous composition of the present invention such that the obtained tin silver alloy is substantially free of, preferably does not comprise, copper. Thus, in such cases an aqueous composition of the present invention is preferred, wherein the composition is substantially free of, preferably does not comprise, copper ions, preferably is substantially free of, preferably does not comprise, copper ions and bismuth ions.

Preferred is an aqueous composition of the present invention being substantially free of, preferably not comprising, nickel ions, zinc ions, iron ions, lead ions, and aluminium ions.

Preferably, said tin ions and said silver ions are the only depositable metal ions in the aqueous composition. This means that these metal ions are the only metal ions that are deposited in the tin silver alloy. Preferred is an aqueous composition of the present invention, wherein in the aqueous composition the weight of said tin ions and said silver ions in total represents 80 wt.-% to 100 wt.-% of all group 3 to group 15 metal cations in the aqueous composition, based on the total weight of all group 3 to group 15 metal cations in the aqueous composition, preferably at least 90 wt.-%, more preferably at least 95 wt.-%, even more preferably at least 98 wt.-%, most preferably at least 99 wt.-%. Group 3 to 15 refers to the 18 groups in the periodic table of elements.

The aqueous composition of the present invention comprises, besides (a) tin ions and (b) silver ions, (c) at least one (preferably one) first compound (as described throughout the present text) and additionally (d) at least one (preferably one) second compound of formula (II).

The at least one first compound is independently selected from the group consisting of unsubstituted bis(aminophenyl)disulfides, substituted bis(aminophenyl)disulfides, unsubstituted dipyridyldisulfides, and substituted dipyridyldisulfides, preferably is independently selected from the group consisting of unsubstituted bis(aminophenyl)disulfides, substituted bis(aminophenyl)disulfides, and unsubstituted dipyridyldisulfides, more preferably is independently selected from the group consisting of unsubstituted bis(aminophenyl)disulfides and substituted bis(aminophenyl)disulfides, most preferably is independently selected from the group consisting of unsubstituted bis(aminophenyl)disulfides. In the context of the present invention, unsubstituted denotes that no additional substituents (i.e. functional groups) are included, wherein substituted denotes that additional substituents (i.e. functional groups) are present.

In the unsubstituted bis(aminophenyl)disulfides preferably each phenyl moiety comprises a single amino group. Preferably, the unsubstituted bis(aminophenyl)disulfides are selected from the group consisting of 4,4'-diaminodiphenyl disulfide (also called 4,4'-dithiodianiline) and 2,2'-diaminodiphenyl disulfide (also called 2,2'-dithiodianiline). More preferred is an aqueous composition of the present invention, wherein the at least one first compound is 2,2'-diaminodiphenyl disulfide. Most preferred is an aqueous composition of the present invention, wherein 2,2'-diaminodiphenyl disulfide is the only first compound.

The unsubstituted dipyridyldisulfides are preferably selected from the group consisting of 4,4'-dipyridyldisulfide and 2,2'-dipyridyldisulfide.

Preferred is an aqueous composition of the present invention, wherein the substituted bis(aminophenyl)disulfides and substituted dipyridyldisulfides have at least one substituent independently selected from the group consisting of C1 to C4 alkyl, C1 to C4 alkoxy, hydroxyl, sulfhydryl, carboxyl, amino, nitro, and halide.

In case of substituted bis(aminophenyl)disulfides an amino substituent denotes a second amino group in at least one of the two phenyl moieties.

In particular preferred is an aqueous composition of the present invention, wherein the substituted bis(aminophenyl)disulfides have at least one substituent independently selected from the group consisting of C1 to C4 alkyl, C1 to C4 alkoxy, hydroxyl, sulfhydryl, carboxyl, amino, nitro, and halide, preferably selected from the group consisting of C1 to C3 alkyl, C1 to C4 alkoxy, hydroxyl, and sulfhydryl, more preferably selected from the group consisting of C1 to C3 alkyl, C1 to C3 alkoxy, and hydroxyl.

In particular preferred is an aqueous composition of the present invention, wherein the substituted dipyridyldisulfides have at least one substituent independently selected from the group consisting of C1 to C4 alkyl, C1 to C4 alkoxy, hydroxyl, sulfhydryl, carboxyl, amino, nitro, and halide, preferably selected from the group consisting of C1 to C3 alkyl, C1 to C4 alkoxy, hydroxyl, sulfhydryl, and amino, more preferably selected from the group consisting of C1 to C3 alkyl, C1 to C3 alkoxy, hydroxyl, and amino.

Even more preferred is an aqueous composition of the present invention, wherein the substituted dipyridyldisulfides have at least one substituent independently selected from the group consisting of methoxy, ethoxy, methyl, ethyl, hydroxyl, and amino.

Most preferably the substituted dipyridyldisulfides have at least one amino substituent.

Preferred is an aqueous composition of the present invention, wherein the total concentration of all first compounds is in the range from 1 mmol/L to 100 mmol/L, based on the total volume of the aqueous composition, preferably from 5 mmol/L to 80 mmol/L, more preferably from 10 mmol/L to 60 mmol/L, even more preferably from 15 mmol/L to 50 mmol/L, most preferably from 20 mmol/L to 40 mmol/L. Preferably, the total concentration as defined above is formed by only one first compound, most preferably by 2,2'-diaminodiphenyl disulfide (2,2'-dithiodianiline). If the total concentration is significantly below 1 mmol/L or significantly above 100 mmol/L undesired variations in the tin silver alloy are frequently observed. Furthermore, in many cases issues with the bath stability were observed.

The at least one second compound of formula (II) comprises one or more than one, preferably one, sulfhydryl group (SH group) in residue X.

In the compound of formula (II), X denotes a C1 to C10 alkyl moiety comprising said one or more than one, preferably one, sulfhydryl group, preferably a C1 to C8 alkyl moiety, more preferably a C1 to C6 moiety, even more preferably a C1 to C5 alkyl moiety, most preferably a C1 to C4 alkyl moiety, each comprising said one or more than one, preferably one, sulfhydryl group. For example, if X is a C1 alkyl moiety comprising one sulfhydryl group, X denotes -CH₂-SH.

Among said C1 to C10 alkyl moiety, alkyl moieties with three or more than three carbon atoms are linear or branched, preferably linear. Linear alkyl moieties are preferably covalently connected with the nitrogen atom in formula (II) via a terminal carbon atom in the linear alkyl moiety. Thus, linear alkyl moieties are preferably n-alkyl moieties.

In the compound of formula (II), R¹ denotes hydrogen, methyl, ethyl, linear C3 to C5 alkyl, branched C3 to C5 alkyl, unsubstituted phenyl, substituted phenyl, unsubstituted benzyl, or substituted benzyl, preferably R¹ denotes hydrogen, methyl, ethyl, linear C3 to C5 alkyl, or branched C3 to C5 alkyl, more preferably R¹ denotes hydrogen, methyl, ethyl, or linear C3 to C5 alkyl, most preferably R¹ denotes methyl or ethyl. In the context of the present invention, branched C3 alkyl denotes its iso-form.

In the compound of formula (II), R² denotes methyl, ethyl, linear C3 to C5 alkyl, branched C3 to C5 alkyl, unsubstituted phenyl, substituted phenyl, unsubstituted benzyl, or substituted benzyl, preferably R² denotes methyl, ethyl, linear C3 to C5 alkyl, or branched C3 to C5 alkyl, more preferably R² denotes methyl, ethyl, or linear C3 to C5 alkyl, most preferably R² denotes methyl or ethyl.

Preferred substituents in said substituted phenyl and substituted benzyl are independently selected from the group consisting of hydroxyl, C1 to C3 alkyl, C1 to C3 alkoxy, amino, nitro, and carboxyl.

The at least one second compound of formula (II) serves as complexing agent in the aqueous composition of the present invention. Preferred is an aqueous composition of the present invention, wherein compounds of formula (II) are the only complexing agents in the composition. It is in particular preferred that the aqueous composition of the present invention is substantially free of, preferably does not comprise, glycine, cysteine, and glutathione, more preferably is substantially free of, preferably does not comprise, amino acids with at least one sulfhydryl group and peptides with at last one sulfhydryl group, most preferably is substantially free of, preferably does not comprise, amino acids and peptides at all. Own experiments indicate that amino acids and peptides have negative influence on the shelf life of the aqueous composition of the present invention, finally causing stability problems. In some cases it has been observed that the shelf life does not go beyond six month, which is not desired. In contrast, a shelf life exceeding six month is desired and compounds of formula (II) do not negatively affect the shelf life, preferably resulting in a shelf life of more than six month.

In the aqueous composition of the present invention, compounds of formula (II) surprisingly serve a second advantage. Typically, during utilization of the aqueous composition of the present invention, compounds of the at least one first compound get reduced, which results in their monomerization. This monomerization is basically desired. Usually this results in a very unpleasant odor due to the aromatic ring with a sulfhydryl group. However, in the context of the present invention it has been observed that compounds of formula (II) reduce compounds of the at least one first compound only to such an extent that unpleasant odors are largely prevented. Instead a progressive and self-regulated reducing is obtained such that the total amount of monomeric first compounds is kept very low but sufficiently high to ensure operational capabilities of the aqueous composition. This is advantageous for people working in close proximity to a respective composition.

Therefore, the combination of the at least one first compound and the at least one second compound of formula (II) results in a number of unexpected advantages.

Preferred is an aqueous composition of the present invention, wherein the at least one second compound of formula (II) is a compound of formula (Ila) wherein independently
R¹ denotes hydrogen, methyl, ethyl, linear C3 to C5 alkyl, branched C3 to C5 alkyl, unsubstituted phenyl, substituted phenyl, unsubstituted benzyl, or substituted benzyl, preferably R¹ denotes hydrogen, methyl, ethyl, linear C3 to C5 alkyl, or branched C3 to C5 alkyl, more preferably R¹ denotes hydrogen, methyl, ethyl, or linear C3 to C5 alkyl, most preferably R¹ denotes methyl or ethyl,
R² denotes methyl, ethyl, linear C3 to C5 alkyl, branched C3 to C5 alkyl, unsubstituted phenyl, substituted phenyl, unsubstituted benzyl, or substituted benzyl, preferably R² denotes methyl, ethyl, linear C3 to C5 alkyl, or branched C3 to C5 alkyl, more preferably R² denotes methyl, ethyl, or linear C3 to C5 alkyl, most preferably R² denotes methyl or ethyl, and
n denotes 1, 2, 3, or 4, preferably n denotes 1, 2 or 3.

In the context of the present invention, linear C3 to C5 alkyl and branched C3 to C5 alkyl preferably and explicitly includes n-propyl, iso-propyl, n-butyl, iso-butyl, sec-butyl, tert-butyl, n-pentyl, 2-methylbutan-2-yl, 2,2-dimethylpropyl, 3-methylbutyl, pentan-2-yl, pentan-3-yl, 3-methylbutan-2-yl, and 2-methylbutyl.

Most preferred is a composition of the present invention, wherein the at least one second compound of formula (II) is 2-(dimethylamino)ethanethiol.

In the aqueous composition of the present invention, compounds of formula (II) are preferably positively charged at the nitrogen atom due to the preferred highly acidic pH (for pH see details above in the text).

Preferred is an aqueous composition of the present invention, wherein the total concentration of all said second compounds of formula (II) is in the range from 5 mmol/L to 100 mmol/L, based on the total volume of the aqueous composition, preferably from 8 mmol/L to 80 mmol/L, more preferably from 10 mmol/L to 60 mmol/L, even more preferably from 15 mmol/L to 50 mmol/L, most preferably from 20 mmol/L to 40 mmol/L. Preferably, the total concentration as defined above is formed by only one second compound, most preferably by only 2-(dimethylamino)ethanethiol. If the total concentration is significantly below 5 mmol/L, silver ions are not sufficiently complexed and undesired plate out is frequently observed.

Preferred is an aqueous composition of the present invention, wherein the molar ratio of all first compounds to all second compounds is in the range from 10:1 to 1:10, preferably in the range from 7:1 to 1:7, more preferably in the range from 5:1 to 1:5, even more preferably in the range from 4:1 to 1:4, most preferably in the range from 3:1 to 1:3, even most preferably in the range from 2:1 to 1:2. If the molar ratio is significantly above 10:1 or significantly below 1:10 the stability of the aqueous composition is in some cases negatively affected. Furthermore, in some cases in the tin silver alloy the total amount of silver was negatively affected, leading to a tin silver alloy comprising too high or too little amounts of silver.

The aqueous composition of the present invention preferably comprises further compounds.

Preferred is an aqueous composition of the present invention furthermore comprising
(e) at least one organic acid anion, preferably an alkyl sulfonic acid anion, most preferably methane sulfonic acid anions.

Said at least one organic acid anion is preferably obtained from the source of tin ions and/or the source of silver ions.

Also preferably, said at least one organic acid anion is obtained from an organic acid, preferably from at least one alkyl sulfonic acid, most preferably from methane sulfonic acid.

Most preferably, said at least one organic acid anion is obtained from the source of tin ions, the source of silver ions, and an organic acid. In such a case, the aqueous composition of the present invention preferably contains only one type of organic acid anion, which is very preferred. Therefore, most preferred is an aqueous composition of the present invention, wherein in the composition alkyl sulfonate, preferably methane sulfonate, is the only organic acid anion. This provides a number of advantages because solubility of metal ions is typically high in the presence of alkyl sulfonic acids. Furthermore, undesired oxidation of tin (II) ions to tin (IV) ions is significantly reduced. In addition it has been observed that the corrosive effect of alkyl sulfonic acids is reduced compared to strong inorganic acids.

Alkyl sulfonic acids are preferred acids because they serve as optimal pH adjuster and typically result in a very strong acidic pH. If other organic acid anions are utilized, preferably acetate, oxalate, and citrate, either as organic acid or in the source of tin ions and/or silver ions, an additional strong acid is usually needed to obtain the preferred strong acidic pH, for example strong inorganic acids, which include additional inorganic anions. This is less preferred, e.g. for the reasons stated above. Thus, preferred is an aqueous composition of the present invention, wherein the composition is substantially free of, preferably does not comprise, inorganic acids. Instead strong organic acids are preferred in the composition of the present invention.

Preferred is an aqueous composition of the present invention, wherein in the aqueous composition the total concentration of all organic acid anions is in the range from 0.5 mol/L to 4.0 mol/L, based on the total volume of the aqueous composition, preferably from 0.6 mol/L to 2.5 mol/L, more preferably from 0.7 mol/L to 2 mol/L, even more preferably from 0.8 mol/L to 1.5 mol/L, most preferably from 0.9 mol/L to 1.3 mol/L. Preferably, the total concentration as defined above is formed by only one type of organic acid anions, more preferably by only alkyl sulfonates, most preferably by only methane sulfonate. If the total concentration is significantly exceeding 4.0 mol/L the composition is not sufficiently stable anymore. Furthermore, a too high total concentration creates severe issues or even damages on the substrate. If the total concentration is significantly below 0.5 mol/L an insufficient conductivity of the aqueous composition is usually obtained.

In order to increase the wettability, the aqueous composition of the present invention preferably comprises at least one surfactant. The kind of surfactant is not particularly limited. Thus, preferred is an aqueous composition of the present invention furthermore comprising
(f) at least one surfactant, preferably selected from the group consisting of nonionic surfactants, amphoteric surfactants, cationic surfactants, and anionic surfactants, preferably nonionic surfactants and cationic surfactants, more preferably alkoxylated cationic surfactants and polyether nonionic surfactants, even more preferably alkylene oxide co-polymers and alkoxylated amines, most preferably ethylene oxide/propylene oxide co-polymers and ethoxylated amines.

Preferred is an aqueous composition of the present invention, wherein the total concentration of all surfactants is in the range from 0.1 g/L to 20 g/L, based on the total volume of the aqueous composition, preferably from 0.4 g/L to 10 g/L, more preferably from 0.6 g/L to 8 g/L, most preferably from 1 g/L to 5 g/L. If the total concentration is significantly below 0.1 g/L in many cases the wettability is insufficient. If the total concentration is significantly exceeding 20 g/L it is often observed that undesired foam is formed.

In order to avoid or at least to suppress foaming, the aqueous composition of the present invention furthermore preferably comprises, at least in many cases, at least one anti-foam agent.

The aqueous composition of the present invention preferably comprises tin (II) ions. However, tin (II) ions are susceptible to oxidation, which results in tin (IV) ions. Such an oxidation is not desired because it promotes precipitation of tin (IV) species, such as tin (IV) oxide. To avoid oxidation, an anti-oxidizing agent is preferably utilized. Thus, preferred is an aqueous composition of the present invention furthermore comprising
(g) at least one anti-oxidizing agent, preferably selected from the group consisting of compounds comprising a hydroxylated ring moiety, most preferably selected from the group consisting of catechol, hydroquinone, resorcinol, phenolsulfonic acids, ascorbic acid, and naptholsulfonic acids.

Preferred hydroxylated ring moieties are hydroxylated aromatic compounds, more preferably benzene diols, even more preferably selected from the group consisting of catechol, hydroquinone, and resorcinol, most preferably selected from the group consisting of resorcinol and hydroquinone. Most preferred is an aqueous composition of the present invention, wherein the at least one anti-oxidizing agent is resorcinol, more preferably resorcinol is the only anti-oxidizing agent in the aqueous composition of the present invention. Anti-oxidizing agents as defined above are strong enough to avoid oxidation of tin (II) ions to tin (IV) ions without reducing tin (II) ions to metallic tin.

The aqueous composition of the present invention is preferably for electrolytically depositing a tin silver alloy and is preferably not for electroless deposition.

Preferred is an aqueous composition of the present invention, wherein the total concentration of all anti-oxidizing agents is in the range from 1.0 mmol/L to 100 mmol/L, based on the total volume of the aqueous composition, preferably from 2.0 mmol/L to 70 mmol/L, more preferably from 4.0 mmol/L to 40 mmol/L, even more preferably from 5.0 mmol/L to 20 mmol/L, most preferably from 6.0 mmol/L to 15 mmol/L. Preferably, the total concentration as defined above is formed by only one type of anti-oxidizing agent, more preferably by only benzene diols, most preferably by only resorcinol. If the total concentration as defined above is significantly exceeding 100 mmol/L in many cases it is observed that the plating performance is insufficient. If the total concentration is significantly below 1.0 mmol/L oxidation of tin (II) ions to insoluble tin (IV) species is not sufficiently prevented and undesired precipitation can be observed in some cases

If the at least one anti-oxidizing agent is known as a typical anti-oxidizing agent, the amount of such a compound is preferably counted among the above mentioned total concentration of all anti-oxidizing agents. In particular, if the at least one anti-oxidizing agent is an organic acid and comprises a hydroxylated ring moiety, the amount of said compound is counted among above mentioned total concentration of all anti-oxidizing agents.

As mentioned above, the present invention also refers to a method for electrolytically depositing a tin silver alloy onto a substrate, the method comprising the steps
(A) providing the substrate,
(B) providing an aqueous composition according to the present invention, preferably as described above as being preferred,
(C) contacting said substrate with said aqueous composition and supplying an electrical current such that said tin silver alloy is electrolytically deposited onto the substrate.

The above mentioned regarding the aqueous composition of the present invention applies likewise to the method of the present invention.

In step (A) of the method of the present invention, the substrate is provided, preferably a conductive substrate. In some cases, preferred is a method of the present invention, wherein the substrate is a semiconductor base substrate, preferably comprising a conductive or semi-conductive layer thereon. Such a conductive or semi-conductive layer is also often referred to as seed layer. The kind of seed layer is not particularly restricted. A most preferred seed layer is a copper seed layer.

The substrate preferably is or comprises at least one metalloid and/or gallium, more preferably is or comprises at least one element selected from the group consisting of silicon, germanium, and gallium, most preferably is or comprises silicon. If the substrate is not in itself sufficiently conductive, it preferably comprises above mentioned conductive or semi-conductive layer.

Most preferred is a method of the present invention, wherein the substrate is a wafer, preferably a wafer comprising a conductive or semi-conductive layer thereon, most preferably comprising a copper seed layer.

In other cases, preferred is a method of the present invention, wherein the substrate is a non-conductive substrate, preferably a substrate being or comprising glass or plastic. In such a case, the substrate preferably comprises already at least partly a conductive seed layer, or a conductive seed layer is deposited in a subsequent processing step.

Preferred is a method of the present invention, wherein the substrate (as defined before) comprises a plurality of individual structural features. Preferred is a method of the present invention, wherein the substrate comprises a plurality of metal features, preferably a plurality of metal pillars and/or areas with at least one metal layer, more preferably a plurality of copper pillars and/or areas with at least one copper layer.

Preferably, the metal features have an aspect ratio in the range from 1:40 to 15:1 (height:width), preferably in the range from 1:30 to 10:1, more preferably in the range from 1:20 to 7:1. Metal pillars and copper pillars, respectively, have a preferred aspect ratio in the range from 1:1 to 10:1, more preferably in the range from 1:1 to 7:1. Metal bumps and copper bumps, respectively, have a preferred aspect ratio in the range from 1:40 to 1:1, preferably in the range from 1:30 to 1:10. In the context of the present invention, individual structural features and metal features, respectively, include individual geometrical forms such as pillars, spots and areas, which are accessible for tin silver alloy deposition by means of the method of the present invention.

Preferred is a method of the present invention, wherein said metal pillars and copper pillars, respectively, have a cylindrical shape. Preferably, said metal pillars and copper pillars, respectively, have a height in the range from 3 µm to 100 µm, preferably from 5 µm to 90 µm, more preferably from 9 µm to 80 µm, even more preferably from 15 µm to 70 µm, most preferably from 20 µm to 70 µm. Preferably, said metal pillars and copper pillars, respectively, have a width in the range from 5 µm to 100 µm, preferably from 10 µm to 80 µm, more preferably from 10 µm to 30 µm.

In the method of the present invention said metal bumps and copper bumps, respectively, can have any shape; preferably a cylindrical, polygonal, and/or rectangular shape.

Preferably, the metal bumps and copper bumps, respectively, have a height in the range from 0.5 µm to 50 µm, preferably from 1 µm to 30 µm, more preferably from 2 µm to 25 µm, even more preferably from 3 µm to 20 µm, most preferably from 4 µm to 15 µm. Preferably, bumps have a width of at least 50 µm, preferably of at least 80 µm, more preferably of at least 100 µm.

In step (B) an aqueous composition of the present invention, preferably as described throughout the text as being preferred, is provided, typically in a tank for electrolytic metal deposition.

In step (C) of the method of the present invention the tin silver alloy is electrolytically deposited onto the substrate. Step (C) requires that the substrate is sufficiently conductive in order to electrolytically deposit the tin silver alloy. Either the substrate provided in step (A) is already sufficiently conductive or the substrate provided in step (A) is processed in subsequent steps such that it is sufficiently conductive prior to step (C). Thus, the substrate in step (C) preferably comprises at least one conductive or semi-conductive layer such that the tin silver alloy is electrolytically deposited thereon. Preferably, the at least one conductive or semi-conductive layer is a conductive metallic, conductive semi-metallic, or conductive non-metallic layer. Most preferably it is a conductive metallic layer, preferably a metallic copper layer, typically a copper seed layer.

A method of the present invention is preferred, wherein in step (C) the tin silver alloy is deposited as solder caps on pillars and/or as solder bumps.

In the method of the present invention, the substrate is operated as a cathode in order to deposit the tin silver alloy in step (C).

Preferred is a method of the present invention, wherein the electrical current is a direct current, preferably with a cathodic current density in the range from 1 A/dm² to 100 A/dm², more preferably with a cathodic current density in the range from 3 A/dm² to 70 A/dm², most preferably with a cathodic current density in the range from 5 A/dm² to 50 A/dm². In some cases it is preferred that the direct current in step (C) is not supplemented by current pulses. This means that preferably in step (C) the direct current is the only electrical current.

Own experiments show that in particular at comparatively high current densities the method of the present invention gives excellent results. This means that at such current densities excellent and very uniform tin silver alloys are deposited and additionally the number of dendrites is impressively low. This is in particular the case compared to compositions comprising amino acids with at least one sulfhydryl group, e.g. cysteine (see examples below). Therefore, particular preferred is a method of the present invention, wherein the electrical current comprises a direct current with a cathodic current density in the range from 10 A/dm² to 40 A/dm², more preferably in the range from 12 A/dm² to 35 A/dm².

A method of the present invention is preferred, wherein in step (C) the contacting and supplying of electrical current is carried out for 3 seconds to 400 min, preferably for 5 seconds to 200 min, most preferably for 6 seconds to 100 min. If the contacting is carried out for significantly less than 3 seconds typically an incomplete tin silver alloy is deposited and the uniformity of the solder caps is insufficient.

In step (C) of the method of the present invention, preferably a tin silver alloy layer is deposited, preferably with a layer thickness in the range from 1 µm to 150 µm, more preferably in the range from 4 µm to 100 µm, even more preferably in the range from 7 µm to 90 µm, most preferably in the range from 10 µm to 80 µm.

Preferred is a method of the present invention, wherein the silver content in the electrolytically deposited tin silver alloy is in the range from 0.1 wt-% to 10 wt-%, based on the total weight of the electrolytically deposited tin silver alloy, preferably is in the range from 0.5 wt-% to 5 wt-%, most preferably is in the range from 1.5 wt-% to 3.5 wt-%. Most preferably the rest of the tin silver alloy is tin. Thus, the major metal in the tin silver alloy is tin. As a result, a method of the present invention is preferred, wherein the tin content in the electrolytically deposited tin silver alloy is at least 60 wt-%, based on the total weight of the electrolytically deposited tin silver alloy, preferably at least 70 wt-%, more preferably at least 80 wt-%, even more preferably at least 90 wt-% or at least 95 wt.-%, most preferably at least 96.5 wt-%, and even most preferably at least 98.5 wt-% or at least 99.5 wt.-%. A tin silver alloy as described above is very much desired and suitable for solder caps on pillars and as solder bumps because of its excellent solderability.

Only in some cases a method of the present invention is preferred, wherein the tin silver alloy comprises copper.

In most cases it is very preferred that the tin silver alloy obtained with the method of the present invention is not a ternary alloy, more preferably not a tin silver copper alloy. Preferably, the tin silver alloy is substantially free of, preferably does not comprise, one, more than one or all elements of the group consisting of zinc, nickel, iron, copper, bismuth, aluminium, and lead. In particular, the tin silver alloy obtained with the method of the present invention is substantially free of, preferably does not comprise, lead.

Preferred is a method of the present invention, wherein in step (C) the aqueous composition has a temperature in the range from 5°C to 90°C, preferably in the range from 15°C to 60°C, more preferably in the range from 20°C to 50°C, most preferably in the range from 22 °C to 40°C. If the temperature is significantly below 5°C no adequate deposition speed is obtained. If the temperature is significantly above 90°C undesired evaporation and bath instability occurs.

The present invention also refers to a use of the aqueous composition of the present invention for electrolytically depositing tin silver alloy solder bumps or tin silver alloy solder caps onto metal pillars, preferably for electrolytically depositing tin silver alloy solder caps onto copper pillars. The aforementioned regarding the aqueous composition of the present invention and the method of the present invention, respectively, applies likewise to the aforementioned use.

The present invention is described in more detail by the following non limiting examples.

### Examples

1. Aqueous composition for depositing a tin silver alloy:

   In a first step different aqueous compositions are prepared as follows:
   1.1 Aqueous composition E-1 (according to the present invention):
      Aqueous composition E-1 according to the present invention comprises 45 g/L tin(II) ions, 1 g/L silver(I) ions, approximately 1 mol/L methane sulfonic acid, approximately 10 mmol/L resorcinol, 20 mmol/L to 40 mmol/L 2,2'-dithiodianiline, 20 mmol/L to 40 mmol/L 2-(dimethylamino)ethanethiol, and ethylene oxide/propylene oxide co-polymers and ethoxylated amines as surfactants. The pH is approximately 0.
   1.2 Comparative aqueous composition C-1 (not according to the present invention):
      For comparative purposes, comparative aqueous composition C-1 comprises 40 g/L tin(II) ions, 1 g/L silver (I) ions, approximately 1 mol/L methane sulfonic acid, approximately 5 mmol/L hydroquinone, 10 mmol/L to 20 mmol/L 2,2'-dithiodianiline, approximately 20 mmol/L cysteine, and surfactants. The pH is approximately 0. Comparative aqueous composition C-1 represents prior art JP 2006-265573 A.
2. Method for electrolytically depositing a tin silver alloy onto a substrate (deposition experiment):
   In a second step depositions are carried out and a tin silver alloy is deposited in each deposition experiment.

As substrates silicon-based wafer coupons, rendered conductive by means of an approximately 500 nm copper seed layer, each comprising nine dies with a plurality of cylindrical copper pillars (height: 10 µm) were provided. The copper pillars were formed within a respective photoresist. Without removing the photoresist, tin silver alloys were deposited on top of the copper pillars to form respective solder caps. As a result, copper pillars with tin silver solder caps were obtained.

For that, 1000 ml of a respective aqueous composition prepared in the first step was provided.

Subsequently, the respective substrates were immersed into the respective composition for varying contact times according to the supplied current density such that in each case an approximately 15 µm tin silver solder cap was deposited (immersion for 60 seconds to 120 seconds depending on applied current density). The temperature of each composition was 25°C and stirring was set to 300 rpm. After each deposition experiment the number and average area of dendrites as well as the uniformity of the solder caps were determined. The parameters for each deposition experiment and the respective results are summarized in Table 1.

**Table 1, parameters and results of deposition experiments**

| Aqueous composition | Current density [A/dm²] | Number of dendrites | Average area of dendrites [µm²] | WIP* [%] | WID** [%] |
|---|---|---|---|---|---|
| E-1 | 15 | < 10 | < 70 | 11 | 8 |
| | 20 | < 10 | < 140 | 13 | 10 |
| | 30 | < 10 | < 190 | 16 | 11 |
| C-1 | 15 | > 600 | > 4000 | 11 | 10 |
| | 20 | > 1000 | > 14000 | 72 | 79 |
| | 30 | > 900 | > 17000 | 48 | 61 |

| | | | | | |
|---|---|---|---|---|---|
| * within pillar non-uniformity ** within die non-uniformity (nine pillars from each die were evaluated) | | | | | |

Table 1 shows that in a deposition experiment utilizing the aqueous composition E-1 the number of dendrites is insignificant, even at comparatively high current densities such as 30 A/dm². This is also observed for the average area of dendrites, which is significantly higher in comparative aqueous composition C-1.

The number of dendrites and the average area of dendrites were determined by a light microscope (Olympus LEXT OLS4000) using software "Olympus Stream Enterprise Desktop 2.2".

The benefit of the aqueous composition of the present invention is furthermore demonstrated in Fig. 1 and Fig. 2, wherein Fig. 1 shows the result utilizing aqueous composition E-1 and Fig. 2 the result of comparative aqueous composition C-1, both at 30 A/dm². In Fig. 1 almost no dendrites are present, wherein in Fig. 2 significantly more dendrites can be seen.

Furthermore, copper pillars with solder caps, obtained with aqueous composition E-1 exhibit a higher uniformity compared to respective capped copper pillars obtained with comparative aqueous composition C-1, in particular at a current density of 30 A/dm². This can be seen by parameters WIP and WID, which are well known in this technical field.

The same improvement has been observed with copper bumps instead of copper pillars (data not shown).

### 3. Complexing properties determined by titration experiments:

In order to evaluate the complexing properties of various compounds for silver ions several titrations were carried out. The results are summarized in Fig. 3.

The titrations were performed as follows:
In a first step an aqueous stock solution (concentration of complexing compound: 50 g/L) comprising the respective compound(s) for silver ions was prepared.

In a second step, portions from the stock solution were added stepwise to a titration solution comprising silver methanesulfonate (concentration corresponding to 1 g/L Ag (I) ions) and a silver rotating disk electrode (RDE) (1000 rpm). The change in overpotential upon adding portions from the stock solution was determined in reference to a reference electrode. The temperature of the titration solution was 25°C.

Fig. 3 shows that the complexing properties vary significantly among the tested compounds.

Compound A alone (2,2'-dithiodianiline) does not provide any significant complexing properties. The overpotential remains almost zero in the range from 0 g/L to 6 g/L of compound A.

Compound B alone (2-(dimethylamino)ethanethiol) shows significant complexing properties toward silver ions. According to Fig. 3, a maximum overpotential of approximately -250 mV was obtained at approximately 3 g/L compound B.

Similar to compound B, compound D alone (glutathione) shows significant complexing properties and a similar maximum overpotential of approximately -250 mV. However, compared to compound B, compound D is less strongly forming respective complexes. This can be seen in the higher concentration of compound D which is required in order to obtain an overpotential especially in the range from -50 mV to -200 mV. This means that compound D is less effective than compound B at lower concentrations. Furthermore, as an organic compound, glutathione in some cases suffers the disadvantage that it is not sufficiently stable over time in respective aqueous compositions (shelf-life).

Compound C alone (L-cysteine) also shows significant complexing properties towards silver ions and is a typical complexing compound in known compositions (compare JP 2006-265573 A). Fig. 3 shows that compound C is a very capable complexing compound. A maximum of approximately -250 mV is already obtained at comparatively low concentrations of less than 2 g/L. Generally, if complex formation takes place at already very low concentrations the working concentration in a respective aqueous composition is typically also low. Under such circumstances maintaining this low working concentration is challenging and requires very sensitive analytical tools, which is usually not desired.

Compound E also shows a maximum overpotential of approximately -250 mV, and, thus, in this regard is very similar compared to compound B, C, and D. In contrast, compound E very quickly forms strong complexes. This is seen in the fact that at already 1 g/L almost the maximum overpotential is obtained. Although compound D is very capable in forming complexes the working concentration is typically too low and maintaining it in a respective aqueous composition is demanding.

The combinations of A and B as well as of A and C are the only means to obtain very strong complexes. In each case a maximum overpotential of approximately -400 mV is obtained. Such strong complex formation is desired in order to avoid undesired plate out of silver. Plate out typically occurs if silver ions are insufficiently complexed such that either insoluble silver species precipitate in the aqueous composition or silver is deposited too quickly on a respective substrate even in the absence of an electrical current. However, only the combination A and B additionally shows a desired working concentration range to obtain an overpotential in the range from -250 mV to -400 mV. Furthermore, the combination A and C suffers the disadvantage that respective solder caps are more susceptible to dendrite formation (compare item 2 above). In the stock solutions of combinations A and B and A and C, respectively, compound A was present in an approximately equimolar amount compared to 50 g/L of compound B and C, respectively. The total concentration of compound A in the stock solution is identical to the concentration of compound A for combinations A and B and A and C, respectively.

## Claims

1. An aqueous composition for depositing a tin silver alloy, the composition comprising
(a) tin ions,
(b) silver ions,
(c) at least one first compound independently selected from the group consisting of unsubstituted bis(aminophenyl)disulfides, substituted bis(aminophenyl)disulfides, unsubstituted dipyridyldisulfides, and substituted dipyridyldisulfides, and
(d) at least one second compound of formula (II) wherein independently
X denotes a C1 to C10 alkyl moiety comprising one or more than one sulfhydryl group,
R¹ denotes hydrogen, methyl, ethyl, linear C3 to C5 alkyl, branched C3 to C5 alkyl, unsubstituted phenyl, substituted phenyl, unsubstituted benzyl, or substituted benzyl, and
R² denotes methyl, ethyl, linear C3 to C5 alkyl, branched C3 to C5 alkyl, unsubstituted phenyl, substituted phenyl, unsubstituted benzyl, or substituted benzyl.

2. The composition of claim 1, wherein the at least one second compound of formula (II) is a compound of formula (IIa) wherein independently
R¹ denotes hydrogen, methyl, ethyl, linear C3 to C5 alkyl, branched C3 to C5 alkyl, unsubstituted phenyl, substituted phenyl, unsubstituted benzyl, or substituted benzyl,
R² denotes methyl, ethyl, linear C3 to C5 alkyl, branched C3 to C5 alkyl, unsubstituted phenyl, substituted phenyl, unsubstituted benzyl, or substituted benzyl, and
n denotes 1, 2, 3, or 4.

3. The composition of claim 1 or 2, wherein the substituted bis(aminophenyl)disulfides and substituted dipyridyldisulfides have at least one substituent independently selected from the group consisting of C1 to C4 alkyl, C1 to C4 alkoxy, hydroxyl, sulfhydryl, carboxyl, amino, nitro, and halide.

4. The composition of any of the aforementioned claims, wherein the composition is acidic, preferably the composition has a pH in the range from -2 to +4, more preferably in the range from -1 to +2, most preferably in the range from -0.5 to +1.2.

5. The composition of any of the aforementioned claims, wherein the molar ratio of all first compounds to all second compounds is in the range from 10:1 to 1:10, preferably in the range from 7:1 to 1:7, more preferably in the range from 5:1 to 1:5, even more preferably in the range from 4:1 to 1:4, most preferably in the range from 3:1 to 1:3, even most preferably in the range from 2:1 to 1:2.

6. The composition of any of the aforementioned claims, wherein the molar ratio of the tin ions to the silver ions is in the range from 200:1 to 5:1, preferably in the range from 150:1 to 10:1, more preferably in the range from 125:1 to 12:1, most preferably in the range from 100:1 to 15:1.

7. The composition of any of the aforementioned claims furthermore comprising
(e) at least one organic acid anion, preferably an alkyl sulfonic acid anion, most preferably methane sulfonic acid anions.

8. The composition of any of the aforementioned claims furthermore comprising
(f) at least one surfactant, preferably selected from the group consisting of nonionic surfactants, amphoteric surfactants, cationic surfactants, and anionic surfactants, preferably nonionic surfactants and cationic surfactants, more preferably alkoxylated cationic surfactants and polyether nonionic surfactants, even more preferably alkylene oxide co-polymers and alkoxylated amines, most preferably ethylene oxide/propylene oxide co-polymers and ethoxylated amines.

9. The composition of any of the aforementioned claims furthermore comprising
(g) at least one anti-oxidizing agent, preferably selected from the group consisting of compounds comprising a hydroxylated ring moiety, most preferably selected from the group consisting of catechol, hydroquinone, resorcinol, phenolsulfonic acids, ascorbic acid, and naptholsulfonic acids.

10. The composition of any of the aforementioned claims, wherein the composition does not comprise copper ions, preferably does not comprise copper ions and bismuth ions.

11. The composition of any of the aforementioned claims, wherein in the aqueous composition the weight of said tin ions and said silver ions in total represents 80 wt.-% to 100 wt.-% of all group 3 to group 15 metal cations in the aqueous composition, based on the total weight of all group 3 to group 15 metal cations in the aqueous composition, preferably at least 90 wt.-%, more preferably at least 95 wt.-%, even more preferably at least 98 wt.-%, most preferably at least 99 wt.-%.

12. A method for electrolytically depositing a tin silver alloy onto a substrate, the method comprising the steps
(A) providing the substrate,
(B) providing an aqueous composition according to any of claims 1 to 11,
(C) contacting said substrate with said aqueous composition and supplying an electrical current such that said tin silver alloy is electrolytically deposited onto the substrate.

13. The method of claim 12, wherein the silver content in the electrolytically deposited tin silver alloy is in the range from 0.1 wt-% to 10 wt-%, based on the total weight of the electrolytically deposited tin silver alloy, preferably is in the range from 0.5 wt-% to 5 wt-%, most preferably is in the range from 1.5 wt-% to 3.5 wt-%.

14. The method of claim 12 or 13, wherein the substrate comprises a plurality of metal features, preferably a plurality of metal pillars and/or areas with at least one metal layer, more preferably a plurality of copper pillars and/or areas with at least one copper layer.

15. Use of an aqueous composition according to any of claims 1 to 11 for electrolytically depositing tin silver alloy solder bumps or tin silver alloy solder caps onto metal pillars, preferably for electrolytically depositing tin silver alloy solder caps onto copper pillars.

## Patentansprüche

1. Eine wässrige Zusammensetzung zum Abscheiden einer Zinn-Silber-Legierung, wobei die Zusammensetzung Folgendes umfasst:
(a) Zinnionen,
(b) Silberionen,
(c) mindestens eine erste Verbindung, die unabhängig aus der Gruppe bestehend aus unsubstituierten Bis(aminophenyl)disulfiden, substituierten Bis(aminophenyl)disulfiden, unsubstituierten Dipyridyldisulfiden und substituierten Dipyridyldisulfiden ausgewählt ist, und
(d) mindestens eine zweite Verbindung der Formel (II) wobei jeweils unabhängig
X eine C1- bis C10-Alkylgruppe bedeutet umfassend eine oder mehr als eine Sulfhydrylgruppe,
R¹ Wasserstoff, Methyl, Ethyl, lineares C3- bis C5-Alkyl, verzweigtes C3- bis C5-Alkyl, unsubstituiertes Phenyl, substituiertes Phenyl, unsubstituiertes Benzyl oder substituiertes Benzyl bedeutet und
R² Methyl, Ethyl, lineares C3- bis C5-Alkyl, verzweigtes C3- bis C5-Alkyl, unsubstituiertes Phenyl, substituiertes Phenyl, unsubstituiertes Benzyl oder substituiertes Benzyl bedeutet.

2. Die Zusammensetzung nach Anspruch 1, wobei es sich bei der mindestens einen zweiten Verbindung der Formel (II) um eine Verbindung der Formel (IIa) wobei unabhängig
R¹ Wasserstoff, Methyl, Ethyl, lineares C3- bis C5-Alkyl, verzweigtes C3- bis C5-Alkyl, unsubstituiertes Phenyl, substituiertes Phenyl, unsubstituiertes Benzyl oder substituiertes Benzyl bedeutet,
R² Methyl, Ethyl, lineares C3- bis C5-Alkyl, verzweigtes C3- bis C5-Alkyl, unsubstituiertes Phenyl, substituiertes Phenyl, unsubstituiertes Benzyl oder substituiertes Benzyl bedeutet und
n 1, 2, 3 oder 4 bedeutet.

3. Die Zusammensetzung nach Anspruch 1 oder 2, wobei die substituierten Bis(aminophenyl)disulfide und substituierten Dipyridyldisulfide mindestens einen Substituenten aufweisen, der unabhängig aus der Gruppe bestehend aus C1- bis C4-Alkyl, C1- bis C4-Alkoxy, Hydroxyl, Sulfhydryl, Carboxyl, Amino, Nitro und Halogenid ausgewählt ist.

4. Die Zusammensetzung nach einem der vorherigen Ansprüche, wobei die Zusammensetzung sauer ist, wobei die Zusammensetzung vorzugsweise einen pH-Wert im Bereich von -2 bis +4, weiter bevorzugt im Bereich von -1 bis +2, ganz besonders bevorzugt im Bereich von -0,5 bis +1,2 aufweist.

5. Die Zusammensetzung nach einem der vorherigen Ansprüche, wobei das Molverhältnis aller ersten Verbindungen zu allen zweiten Verbindungen im Bereich von 10:1 bis 1:10, vorzugsweise im Bereich von 7:1 bis 1:7, weiter bevorzugt im Bereich von 5:1 bis 1:5, noch weiter bevorzugt im Bereich von 4:1 bis 1:4, ganz besonders bevorzugt im Bereich von 3:1 bis 1:3, am meisten bevorzugt im Bereich von 2:1 bis 1:2 liegt.

6. Die Zusammensetzung nach einem der vorherigen Ansprüche, wobei das Molverhältnis der Zinnionen zu den Silberionen im Bereich von 200:1 bis 5:1, vorzugsweise im Bereich von 150:1 bis 10:1, weiter bevorzugt im Bereich von 125:1 bis 12:1, ganz besonders bevorzugt im Bereich von 100:1 bis 15:1 liegt.

7. Die Zusammensetzung nach einem der vorherigen Ansprüche, ferner umfassend
(e) mindestens ein Anion einer organischen Säure, vorzugsweise ein Alkylsulfonsäure-Anion, ganz besonders bevorzugt Methansulfonsäure-Anionen.

8. Die Zusammensetzung nach einem der vorherigen Ansprüche, ferner umfassend
(f) mindestens ein Tensid, das vorzugsweise aus der Gruppe bestehend aus nichtionischen Tensiden, amphoteren Tensiden, kationischen Tensiden und anionischen Tensiden, vorzugsweise nichtionischen Tensiden und kationischen Tensiden, weiter bevorzugt alkoxylierten kationischen Tensiden und nichtionischen Polyethertensiden, noch weiter bevorzugt Alkylenoxid-Copolymeren und alkoxylierten Aminen, ganz besonders bevorzugt Ethylenoxid/Propylenoxid-Copolymeren und ethoxylierten Aminen, ausgewählt ist.

9. Die Zusammensetzung nach einem der vorherigen Ansprüche, ferner umfassend
(g) mindestens ein Antioxidans, das vorzugsweise aus der Gruppe bestehend aus Verbindungen mit einer hydroxylierten Ringeinheit ausgewählt ist und ganz besonders bevorzugt aus der Gruppe bestehend aus Catechol, Hydrochinon, Resorcin, Phenolsulfonsäuren, Ascorbinsäure und Naphtholsulfonsäuren ausgewählt ist.

10. Die Zusammensetzung nach einem der vorherigen Ansprüche, wobei die Zusammensetzung keine Kupferionen umfasst, vorzugsweise keine Kupferionen und keine Bismutionen umfasst.

11. Die Zusammensetzung nach einem der vorherigen Ansprüche, wobei das Gesamtgewicht der Zinnionen und der Silberionen 80 Gew.-% bis 100 Gew.-% aller Metallkationen aus Gruppe 3 bis Gruppe 15 in der wässrigen Zusammensetzung ausmacht, bezogen auf das Gesamtgewicht aller Metallkationen aus Gruppe 3 bis Gruppe 15 in der wässrigen Zusammensetzung, vorzugsweise mindestens 90 Gew.-%, weiter bevorzugt mindestens 95 Gew.-%, noch weiter bevorzugt mindestens 98 Gew.-%, ganz besonders bevorzugt mindestens 99 Gew.-%.

12. Ein Verfahren zum elektrolytischen Abscheiden einer Zinn-Silber-Legierung auf einem Substrat, wobei das Verfahren die folgenden Schritte umfasst:
(A)Bereitstellen des Substrats,
(B)Bereitstellen einer wässrigen Zusammensetzung nach einem der Ansprüche 1 bis 11,
(C)Inkontaktbringen des Substrats mit der wässrigen Zusammensetzung und Zuführen eines elektrischen Stroms derart, dass die Zinn-Silber-Legierung elektrolytisch auf dem Substrat abgeschieden wird.

13. Das Verfahren nach Anspruch 12, wobei der Silbergehalt in der elektrolytisch abgeschiedenen Zinn-Silber-Legierung im Bereich von 0,1 Gew.-% bis 10 Gew.-%, bezogen auf das Gesamtgewicht der elektrolytisch abgeschiedenen Zinn-Silber-Legierung, liegt, vorzugsweise im Bereich von 0,5 Gew.-% bis 5 Gew.-% liegt, ganz besonders bevorzugt im Bereich von 1,5 Gew.-% bis 3,5 Gew.-% liegt.

14. Das Verfahren nach Anspruch 12 oder 13, wobei das Substrat mehrere Metallmerkmale, vorzugsweise mehrere Metallsäulen und/oder Bereiche mit mindestens einer Metallschicht, weiter bevorzugt mehrere Kupfersäulen und/oder Bereiche mit mindestens einer Kupferschicht, umfasst.

15. Verwendung einer wässrigen Zusammensetzung nach einem der Ansprüche 1 bis 11 zum elektrolytischen Abscheiden von Lötperlen aus Zinn-SilberLegierungen oder von Lötkappen aus Zinn-SilberLegierungen auf Metallsäulen, vorzugsweise zum elektrolytischen Abscheiden von Lötkappen aus Zinn-Silber-Legierungen auf Kupfersäulen.

## Revendications

1. Composition aqueuse pour le dépôt d'un alliage d'étain et d'argent, la composition comprenant
(a) des ions étain,
(b) des ions argent,
(c) au moins un premier composé indépendamment choisi dans le groupe constitué par les bis(aminophényl)disulfures non substitués, les bis(aminophényl)disulfures substitués, les dipyridinyldisulfures non substitués, et les dipyridinyldisulfures substitués, et
(d) au moins un deuxième composé de formule (II) dans laquelle indépendamment
X désigne un fragment C₁₋₁₀-alkyle comprenant un ou plus d'un groupe sulfhydryle,
R¹ désigne hydrogène, méthyle, éthyle, C₃₋₅-alkyle linéaire, C₃₋₅-alkyle ramifié, phényle non substitué, phényle substitué, benzyle non substitué, ou benzyle substitué, et
R² désigne méthyle, éthyle, C₃₋₅-alkyle linéaire, C₃₋₅-alkyle ramifié, phényle non substitué, phényle substitué, benzyle non substitué, ou benzyle substitué.

2. Composition selon la revendication 1, l'au moins un deuxième composé de formule (II) étant un composé de formule (IIa) dans laquelle indépendamment
R¹ désigne hydrogène, méthyle, éthyle, C₃₋₅-alkyle linéaire, C₃₋₅-alkyle ramifié, phényle non substitué, phényle substitué, benzyle non substitué, ou benzyle substitué, et
R² désigne méthyle, éthyle, C₃₋₅-alkyle linéaire, C₃₋₅-alkyle ramifié, phényle non substitué, phényle substitué, benzyle non substitué, ou benzyle substitué, et
n désigne 1, 2, 3 ou 4.

3. Composition selon la revendication 1 ou 2, les bis(aminophényl)disulfures substitués et les dipyridinyldisulfures substitués possédant au moins un substituant indépendamment choisi dans le groupe constitué par C₁₋₄-alkyle, C₁₋₄-alcoxy, hydroxyle, sulfhydryle, carboxyle, amino, nitro, et halogénure.

4. Composition selon l'une quelconque des revendications précédentes, la composition étant acide, préférablement la composition possédant un pH dans la plage de -2 à +4, plus préférablement dans la plage de -1 à +2, le plus préférablement dans la plage de -0,5 à +1,2.

5. Composition selon l'une quelconque des revendications précédentes, le rapport molaire de de tous les premiers composés sur tous les deuxièmes composés se situant dans la plage de 10:1 à 1:10, préférablement dans la plage de 7:1 à 1:7, plus préférablement dans la plage de 5:1 à 1:5, encore plus préférablement dans la plage de 4:1 à 1:4, le plus préférablement dans la plage de 3:1 à 1:3, encore le plus préférablement dans la plage de 2:1 à 1:2.

6. Composition selon l'une quelconque des revendications précédentes, le rapport molaire des ions étain aux ions argent se situant dans la plage de 200:1 à 5:1, préférablement dans la plage de 150:1 à 10:1, plus préférablement dans la plage de 125:1 à 12:1, le plus préférablement dans la plage de 100:1 à 15:1.

7. Composition selon l'une quelconque des revendications précédentes comprenant en outre
(e) au moins un anion d'acide organique, préférablement un anion d'acide alkylsulfonique, le plus préférablement des anions d'acide méthanesulfonique.

8. Composition selon l'une quelconque des revendications précédentes comprenant en outre
(f) au moins un tensioactif, préférablement choisi dans le groupe constitué par les tensioactifs non ioniques, les tensioactifs amphotères, les tensioactifs cationiques, et les tensioactifs anioniques, préférablement les tensioactifs non ioniques et les tensioactifs cationiques, plus préférablement les tensioactifs cationiques alcoxylés et les tensioactifs non ioniques de type polyéther, encore plus préférablement les copolymères d'oxyde alkylène et les amines alcoxylées, le plus préférablement les copolymères oxyde d'éthylène/oxyde de propylène et les amines éthoxylées.

9. Composition selon l'une quelconque des revendications précédentes comprenant en outre
(g) au moins un agent antioxydant, préférablement choisi dans le groupe constitué par des composés comprenant un fragment cyclique hydroxylé, le plus préférablement choisi dans le groupe constitué par le catéchol, l'hydroquinone, le résorcinol, les acides phénolsulfoniques, l'acide ascorbique, et les acides naphtolsulfoniques.

10. Composition selon l'une quelconque des revendications précédentes, la composition ne comprenant pas d'ions cuivre, préférablement ne comprenant pas d'ions cuivre ni d'ions bismuth.

11. Composition selon l'une quelconque des revendications précédentes, où dans la composition aqueuse le poids desdits ions étain et desdits ions argent représente au total 80 % en poids à 100 % en poids de tous les cations du groupe 3 au groupe 15 dans la composition aqueuse, sur la base du poids total de tous les cations du groupe 3 au groupe 15 dans la composition aqueuse, préférablement au moins 90 % en poids, plus préférablement au moins 95 % en poids, encore plus préférablement au moins 98 % en poids, le plus préférablement au moins 99 % en poids.

12. Procédé pour le dépôt de façon électrolytique d'un alliage d'étain et d'argent sur un substrat, le procédé comprenant les étapes de
(A) mise à disposition du substrat,
(B) mise à disposition d'une composition aqueuse selon l'une quelconque des revendications 1 à 11,
(C) mise en contact dudit substrat avec ladite composition aqueuse et fourniture d'un courant électrique de sorte que l'alliage d'étain et d'argent est déposé de façon électrolytique sur le substrat.

13. Procédé selon la revendication 12, la teneur en argent dans l'alliage d'étain et d'argent déposé de façon électrolytique se situant dans la plage de 0,1 % en poids à 10 % en poids, sur la base du poids total de l'alliage d'étain et d'argent déposé de façon électrolytique, préférablement se situant dans la plage de 0,5 % en poids à 5 % en poids, le plus préférablement se situant dans la plage de 1,5 % en poids à 3,5 % en poids.

14. Procédé selon la revendication 12 ou 13, le substrat comprenant une pluralité d'éléments métalliques, préférablement une pluralité de piliers et/ou de zones métalliques comportant au moins une couche métallique, plus préférablement une pluralité de piliers et/ou de zones de cuivre comportant au moins une couche de cuivre.

15. Utilisation d'une composition aqueuse selon l'une quelconque des revendications 1 à 11 pour le dépôt de façon électrolytique de bosses de soudure en alliage d'étain et d'argent ou de capuchons de soudure en alliage d'étain et d'argent sur des piliers métalliques, préférablement pour le dépôt de façon électrolytique de capuchons de soudure en alliage d'étain et d'argent sur des piliers de cuivre.
